

March 2, 1948.

W. J. MARENICK

2,436,931

METHOD OF PREVENTING SCALING DURING THE FORGING OF HOLLOW METAL ARTICLES

Filed Aug. 25, 1944

FIG-1



FIG-2



FIG-3



FIG-4



FIG-5



FIG-6



INVENTOR  
William J. Marencik

By Charleswells Hill

## UNITED STATES PATENT OFFICE

2,436,931

## METHOD OF PREVENTING SCALING DURING THE FORGING OF HOLLOW METAL ARTICLES

William J. Marencik, Parma, Ohio, assignor to Thompson Products, Inc., Cleveland, Ohio, a corporation of Ohio

Application August 25, 1944, Serial No. 551,195

5 Claims. (Cl. 29—156.7)

1

This invention relates to a method of preventing scaling during the forging of hollow metal articles, and more particularly to a method of preventing the scaling of the internal surface of a cup-shaped metal blank in forging the same into a hollow head valve.

In making hollow head poppet valves for aircraft or other automotive engines, a cup-shaped metal blank is subjected to a series of hot forging operations to form an elongated solid stem portion and a head portion provided with a cavity therein. One such method is described and claimed in the McBride et al. Patent No. 1,984,751. During the hot forging operations, which are carried out at a sufficiently elevated temperature to cause scale formation, scale forms on the internal surface of the cup-shaped blank and remains on such surface after the forging operations are complete. It has heretofore been a very difficult and expensive task to remove this scale in finishing the hollow head valve for the reception of a coolant, such as metallic sodium. This scale must, however, be completely removed to prevent contamination of the coolant with the scale and also to obtain an efficient rate of heat transfer through the metal of the valve to the coolant contained within the hollow head thereof.

I have now found that the surface of a hollow metal article can be satisfactorily protected from scaling and oxidation during the hot forging thereof from blank forms if the internal surface of the blank itself is sealed against the entrance thereto of air and hot gases during the forging steps. In accordance with my present invention, this is accomplished by applying a metal cap to the open end of the blank and deforming the metal of the blank to secure the cap in place thereon. The cap is so applied and secured in place while the blank is cool and the internal surface thereof entirely free from scale or oxides. Since the cap then remains in place during the subsequent hot forging operations, or other form of heat treatment, the internal surface of the blank has no opportunity to become oxidized, other than through the action of the small amount of air sealed within the blank at the start. This amount of oxidation is not sufficient to be objectionable, but if it should prove to be so, the air in the blank cavity can first be displaced by means of carbondioxide, or other inert gas. Carbondioxide is preferred because being heavier than air, it will displace air if introduced into the blank either in gaseous form, or in the form of solid carbon-dioxide.

As a further protection for the internal sur-

2

faces of the blank during the hot forging operations, the capped end of the blank may be coated with glass-forming ingredients, such as frit, as disclosed in the copending application of myself and Robert E. Ahlf, Serial No. 551,194, filed August 25, 1944. Ordinarily, however, if the metal cap is properly secured in place on the open end of the cup-shaped blank, as by peening over the metal of the blank, a gas-tight seal is thereby provided that prevents the occurrence of scale formation on the internal surface of the blank during the hot forging operations. The metal cap remains in place during the forging or other operations and becomes included in the metal of the blank. Prior to the forming of the finished hollow metal article, the portion of the forged blank that includes the metal of the cap is removed. The internal surface of the article has now been prevented from becoming scaled during all of the operations performed in making the finished article that involve scaling temperatures.

It is therefore an important object of this invention to provide a method of preventing the formation of scale and oxides on the internal surfaces of metal articles during the hot forging of the blanks in the production of such articles.

It is a further important object of this invention to provide a method of preventing scale formation during the hot forging of metal blanks in the manufacture of hollow metal articles, such as hollow head valves and the like, wherein the interior of the blank is sealed by a metal cap while the internal surface thereof is free from scale or oxides, the cap remaining in place during the subsequent hot forging operations to seal the interior of the blank and protect the internal surface thereof until after all operations at elevated temperatures have been completed.

Other and further important objects of this invention will be apparent from the disclosures in the specification and the accompanying drawings.

## On the drawings:

Figure 1 is a longitudinal sectional view of a cup-shaped blank with a metal cap applied to the open end thereof and with a peening hammer in position before striking the end of the blank to peen the metal of the blank about the periphery of the metal cap.

Figure 2 is a view similar to Figure 1 with the peening hammer in the act of performing the peening operation.

Figure 3 is a longitudinal sectional view of a cup-shaped blank with the cap secured in position.

Figure 4 is a longitudinal sectional view of the valve blank in one stage of its manufacture after being subjected to a hot forging step.

Figure 5 is a longitudinal sectional view of the valve blank after being subjected to a further hot forging step that results in closing the stem end of the valve blank.

Figure 6 is a longitudinal sectional view, similar to Figure 3, illustrating the application of a further protective coating over the capped end of the blank.

Although the invention here illustrated and described is applied to the manufacture of hollow head valves, such as aircraft valves, it will be understood that it is similarly applicable to the manufacture of any hollow metal article which is formed from a cup-shaped blank by a series of hot forging operations. In the case of a hollow head valve, these hot forging operations include the use of hammers to reduce the diameter of the blank adjacent its head end and thereby form a neck portion, and also the use of extrusion dies, swaging dies, upsetting dies, and the like. During such hot forging operations, temperatures are used, such as in the neighborhood of about 1,800° to 2,100° F., that would normally cause scale formation on the surfaces of the metal blank. Since these operations are of themselves well known and some of them are described in the McBride et al patent above referred to, they will not be explained in detail here.

The reference numeral 10 indicates generally a cup-shaped blank such as is used in the forming of a hollow head valve. The blank 10 is itself the result of a series of prior operations and comprises an enlarged head portion 11 and a stem portion 12 of slightly reduced diameter. Within the head portion 11 is a head cavity 13 which merges into a stem cavity 14. Prior to the start of the operations about to be described, the valve blank 10 has been machined to leave the internal surface of the head and stem cavities 13 and 14, respectively, clean and free from any scale or oxides.

With the valve blank 10 in the cleaned condition indicated, the open end of the blank is sealed before the blank is subjected to any high temperatures in the course of manufacturing the hollow head valve.

As illustrated in Figures 1 and 2, the open stem end of the blank 10 is recessed, as at 15, to receive a metal cap 16 to provide a seal for the interior of the blank. Said metal blank 16, which may be formed of stainless steel or other suitable metal, is preferably initially dished to give it a convexity upwardly as illustrated in Figure 1. The metal cap 16 is placed in the annular recess 15 and then struck with a peening hammer 17. The bottom face of said hammer 17 is provided with a segmental spherical concave surface 18 centrally and with a surrounding conical recess 19. The action of the hammer 17 is thus to give a segmental spherical contour to the metal cap 16 and to cause the metal of the end of the blank to flow over and around the periphery of the metal cap 16, as at 20. The cap 16 is thereby firmly sealed in place and the internal walls of the blank 10 are sealed against the entrance of air or gases thereinto.

Starting with the capped blank 10 as illustrated in Figure 3, the blank is subjected to a series of hot forging operations as a result of which the blank passes through the stages illustrated in Figures 4 and 5. In one of the hot forging operations, the blank 10 is reduced to provide

a neck 21 and an elongated stem portion 22, also of reduced diameter. The metal cap 16 during this forging step becomes deformed and assumes a slightly angular shape. The shape is of no particular importance except that it indicates the behavior of the metal cap when the blank is subjected to the forging operations to form the neck and stem of reduced diameter. When a stainless steel cap is used, no difficulty is experienced from the cap breaking or rupturing.

In a second forging operation, the valve blank 10 is subjected to an extrusion step that results in closing the stem of the valve to provide an elongated closed stem 23 and a head cavity 24. The metal of the cap 16, now indicated by the reference numeral 16a, is enclosed within the metal of the elongated stem 23. Since the mass of the cap metal 16a is substantially at the extremity of the stem portion, the stem end can be severed, as at the dotted line 25 (Figure 5) to eliminate the cap metal entirely from the finished valve. Subsequent operations beyond those illustrated are carried out to produce the finished valve, but since these operations do not involve temperatures at which scaling would take place, no further protection of the surface of the head cavity 24 is required. The elongated stem 23 is drilled out to permit the introduction of a coolant, such as metallic sodium, into the head cavity 24, and the valve blank otherwise finished in accordance with well known practice.

In the modification of my invention illustrated in Figure 6, in addition to a metal cap 16, the end of the valve blank 10, including said cap 16, is provided with a coating of material, such as frit, capable upon fusing of forming a glassy protective layer 26. To accomplish this, an aqueous suspension of frit is applied to the end of the valve blank 10, as by dipping or spraying, to form a layer 26 thereover. After the end of the blank has been coated with a layer of the aqueous frit suspension, it is subjected to a preliminary heating step, as by heating to about 200° F. to dry the frit coating to form a dry, relatively hard adherent layer 26. During the subsequent hot forging operations, this layer 26 becomes fused to form a glassy protective coating over the entire end of the blank, thus insuring complete protection of the interior wall of the valve blank during the hot forging operations. As before stated, the cap continues to protect the interior as the valve takes shape, because it does not resist deformation but collapses upon itself without breaking the seal. The glassy coating 26, however, protects against the possibility of the metal cap 16 drawing away from the peened over metal bead 20 to produce a leak in the seal.

In accordance with the principles of this invention, therefore, hollow metal articles may be protected against surface oxidation or scaling by the use of either a thin metal cap alone or a metal cap and a protective glassy coating to seal the blank cavity during hot forging operations.

I claim as my invention:

1. In the method of making a hollow head valve in which a cup-shaped blank is subjected to a series of hot forging operations, the improvement whereby scaling of the internal surface of the blank is prevented, which comprises applying an outwardly dished metal cap to the open end of said blank to seal the empty cavity therein, peening the metal of said blank about said cap to secure the same in place and seal the interior of said blank, and subsequently subjecting said blank to hot forging operations.

2. In the method of making a hollow head valve in which a cup-shaped blank is subjected to a series of hot forging operations, the improvement whereby scaling of the internal surface of the blank is prevented which comprises applying an outwardly dished metal cap to the open end of said blank to seal the empty cavity therein, peening the metal of said blank about said cap to secure the same in place and seal the interior of said blank prior to subjecting said blank to hot forging operations, hot forging said blank to form a hollow head, a reduced neck and an elongated solid stem with the metal of said cap included in the end of said stem and removing said stem end that includes the metal of said cap.

3. In the method of making a hollow head valve in which a cup-shaped blank is subjected to a series of hot forging operations, the improvement whereby scaling of the internal surface of the blank is prevented, which comprises applying an outwardly dished metal cap to the open end of said blank, peening the metal of said blank about said cap to secure the same in place and seal the empty interior of said blank prior to subjecting said blank to hot forging operation, hot forging said blank to form a hollow head, a reduced neck and an elongated solid stem with the metal of said cap included in the end of said stem and removing said stem end.

4. In the method of making a hollow head valve from a cup-shaped blank by a series of hot forging operations, the improvement preventing scaling of the internal surface of said blank, which comprises applying an outwardly dished metal cap to the open end of said blank while the internal surface is clean and free from scale,

securing said cap in place by deformation of the metal of said blank to seal the empty interior thereof, subjecting said blank to hot forging operations during which the metal of said cap becomes included within the metal of said blank, and thereafter removing the portion of the blank that includes said cap metal.

5. In the method of making a hollow head valve from a cup-shaped blank by a series of hot forging operations, the improvement preventing scaling of the internal surface of said blank, which comprises applying an outwardly dished metal cap to the open end of said blank to seal the empty cavity therein while the internal surface is clean and free from scale, securing said cap in place by deformation of the metal of said blank, applying a frit coating over said cap to protect the cap end of said blank and to seal the interior thereof, subjecting said sealed blank to hot forging operations during which the metal of said cap becomes included within the metal of said blank, and thereafter removing the portion of the blank that includes said cap metal.

WILLIAM J. MARENICK.

## 25

## REFERENCES CITED

The following references are of record in the file of this patent:

## UNITED STATES PATENTS

| 20 | Number    | Name    | Date           |
|----|-----------|---------|----------------|
|    | 1,364,565 | Lloyd   | Jan. 4, 1921   |
|    | 1,409,562 | Mason   | Mar. 14, 1922  |
|    | 2,005,306 | Wallis  | June 18, 1935  |
| 25 | 2,081,645 | Squires | May 25, 1937   |
|    | 2,093,771 | Colwell | Sept. 21, 1937 |